

Dec. 23, 1941.

W. G. CALKINS ET AL

2,267,372

POWDERED METAL PRODUCT

Filed Sept. 5, 1940



INVENTORS  
WILLIAM G. CALKINS  
ROY E. BLUE AND  
WARD W. MARVIN.

BY  
Gardner, Lind, Peter, Davis  
ATTORNEYS.

## UNITED STATES PATENT OFFICE

2,267,372

## POWDERED METAL PRODUCT

William G. Calkins and Roy E. Blue, Detroit, and  
Ward W. Marvin, Royal Oak, Mich., assignors  
to Chrysler Corporation, Highland Park, Mich.,  
a corporation of Delaware

Application September 5, 1940, Serial No. 355,424

5 Claims. (Cl. 75—22)

Our present invention relates to the formation of articles, such as screen material, from comminuted metal.

The principal object of the invention is to provide screen material of any desired shape, contour, mesh, corrosion resistance, or other characteristics, from metals or alloys of metals by a process comprising comminuting the metals or alloys of metals, then compressing the comminuted particles together in the shape desired and sintering the particles together.

An advantage of the present invention is that any metals or alloys of metals which can be ground into fine particles and agglomerated by heat may be formed into articles such as screen material. A further advantage of the present invention is that screen material may be formed with reinforcing ribs integrally associated therewith, with binding edges integrally formed thereon, or with fancy shapes, contours and mesh characteristics, irregular meshes, or any other feature desired by the designer of the article or screen material.

A further object of the present invention is to form screen material of metals or alloys of metals in mesh sizes which could not be achieved by molten molding processes, and which could only be achieved with considerable difficulty or expense by wire drawing and weaving processes or by drilling or perforating flat sheets.

A further object of the present invention is to provide a method and apparatus for forming screen material having the above characteristics.

These and other objects and advantages of the present invention may be realized from an inspection of the accompanying specification and drawing wherein a preferred form of the article and apparatus is illustrated and described and wherein preferred methods of operation are schematically illustrated and described.

In the drawing, wherein like numerals refer to like parts throughout, Fig. 1 is a view in perspective of a portion of a mold for forming screen material in accordance with the present invention;

Fig. 2 illustrates a step in the operation of forming an article, such as screen material, in accordance with the herein disclosed process and using the mold illustrated in Fig. 1;

Fig. 3 illustrates a further step in the process herein disclosed, showing a portion of a press of utility in accordance with the present disclosure;

Fig. 4 shows a further step in the process here-

in disclosed showing a furnace for sintering the material in the mold;

Fig. 5 discloses an article, such as screen material, formed by the present process and apparatus; and,

Fig. 6 is a sectional view taken substantially along line 6—6 of Fig. 5.

In accordance with our invention we may use any comminuted metal or alloy, such as copper, bronze, brass, nickel, chromium, Monel metal, iron, or any other suitable or desired metal or alloy which is capable of being ground or comminuted in any known manner to a particle size sufficiently smaller than the smallest dimensions

10 of the article to be formed in order that the particles may be compacted into grooves or depressions conforming to the article to be formed. For example, 90% copper in comminuted form may be mixed with 10% tin in comminuted form; or 90% iron and 10% tin in comminuted form may be mixed together; or three or more metals may be so mixed; or various metals may be first alloyed and then comminuted to give the desired proportion of basic metals in alloyed form. It is

15 only necessary that a metal of high melting point constitute the major proportion of the metal present so that the comminuted particles may be sintered at a temperature below the melting point of the metal forming the major proportion of the mass and above the melting point of the metal, or metals, forming the minor proportion of the mass

20 in order that the metal of low melting point may flow around and between the particles of metal of high melting point to sinter the mass into a self-sustaining structure for which the metal of high melting point provides the structural strength and other properties desired. In this regard the metal of low melting point may be

25 tin which would bond together particles of copper or some other metal having a higher melting point, the tin also providing a surface coating for resistance against corrosion; or the metal of low melting point may be copper which would flow around and between particles of a metal of higher melting point, such as iron, to bond the iron particles together and to protect the same from rust

30 and other forms of corrosion. It may be desirable to first alloy the metals in the desired proportion, then to grind or otherwise comminute the alloy, and then to sinter the comminuted alloy particles so that some of the metal of low melting point would sweat out of the alloy sufficiently to form bonding contact with other particles in the mass

35 of material, in which case the articles would com-

prise principally the alloyed metals in a state of alloy having desired properties not obtainable with the use of mixtures of the same metals.

As seen in the drawing, a mold may be provided by shaping a surface 10 of a block of material 11, the mold being formed from a substance which is infusible at the temperatures necessary to sinter the comminuted particles. The substance from which the mold is formed may comprise any of such materials as graphite, stainless steel, ceramic material, or cold rolled steel having a chromium oxide surface protection thereon. The mold is machined or otherwise shaped to conform to the contours of the desired article, the mold in Fig. 1 being shaped to provide intersecting grooves 12 and an edge depression 13. In the illustration, the grooves 12 conform to the shape and mesh size of screen material desired and the edge depression forms a square bead or edge trim around the screen integrally united with the mesh of the screen.

In performing the process of forming articles the depressions in the surface of the mold are filled by heaping a mass of the comminuted material on top of the mold and removing the excess material extending above the depressions in the mold, as by means of moving a straight-edge 15 across a plane surface mold or by otherwise striking off the excess material extending above the mold. The mold with the material in the depressions therein is then placed in a press as shown in Fig. 3 comprising a bed 16 on which the mold is placed and a ram 17 comprising a platen 18 of rubber, or other rubberous material such as chloroprene or Buna rubber, placed in a depression 19 in the ram which is shaped to fit over the edge of the mold. The rubberous material is preferably sufficiently resilient to flow into the depressions of the mold and compress the comminuted particles into intimate contact with each other, but of sufficient surface strength not to be ruptured or punctured by the comminuted particles. If necessary or desirable, the mold may be removed after compression of the mass of comminuted particles and the steps of placing a mass of comminuted material thereon, removing the excess material therefrom and compressing the material in the depressions may be repeated until the material has been built up in the depressions to the desired depth or thickness.

In order to aid in the compression of the particles into a closely knit mass of particles, it is sometimes desirable to add a small proportion of a dry lubricant, such as powdered boric acid, graphite powder, exfoliated vermiculite, or any other dry substance which aids in causing the particles to slide past one another and which is preferably incapable of detracting from the alloy characteristics or the bonding strength of the metals when the mass is sintered. Such a dry lubricant should be added in amounts of from  $\frac{1}{2}\%$  to  $1\frac{1}{2}\%$  of the comminuted metal.

After sufficient powdered material has been compacted into the depressions of the mold, the mold is placed in an oven 20 having a non-oxidizing atmosphere maintained therein at a sintering temperature. The atmosphere may be a reducing atmosphere such as hydrogen, or it may be an inert atmosphere such as ordinary illuminating gas.

The sintering operation is preferably conducted at a temperature between the melting points of the metals of higher and lower melting

points. For example, a mixture of copper and tin may be sintered at an atmosphere of  $1600^{\circ}$  F. to  $1650^{\circ}$  F., the melting point of commercially pure copper being  $1981^{\circ}$  F. and the melting point of commercially pure tin being  $415^{\circ}$  F. The sintering operation is maintained at the stated temperature long enough for the tin to be melted and to flow between the particles of copper to bond the same together and protect the surfaces thereof. In an iron and copper mixture a temperature between the melting point of copper and the melting point of iron, such as  $2200^{\circ}$  F. to  $2500^{\circ}$  F. may be maintained sufficiently long enough to cause the copper to flow between the particles of iron. If an alloy is comminuted and sintered in the mold the temperature is preferably maintained at a temperature below the melting point of the alloy but above the melting point of the metal of lower melting point in the alloy. Thus, Coe bronze, which is  $89\frac{1}{2}\%$  copper and  $10\frac{1}{2}\%$  tin, melts at substantially  $1832^{\circ}$  F., as does gun metal bronze which is 90% copper and 10% tin, and the sintering temperature is preferably maintained in the neighborhood of  $1600^{\circ}$  F. to  $1650^{\circ}$  F., which is considerably below the melting point of the alloy but sufficiently above the melting point of the tin in the alloy to cause some of the tin to sweat out of the alloy and bond the alloy particles together. The sintering oven may be maintained at any temperature above the melting point of the metal of low melting point and below the melting point of the metal of high melting point but preferably should be maintained at a temperature closer to the melting point of the metal of high melting point so that the sintering operation may be more rapidly performed.

An unexpected result of the foregoing process is that very fine mesh screen material formed from particles compacted in an open groove would be expected to have a completely flat surface contour, whereas the fact is that the compressing and sintering operations cause the mesh strand portions to assume a cylindrical or nearly cylindrical shape. An advantage of the foregoing process is that very large sheets of fine mesh screen material may be formed whereas molten molding processes even when conducted at high temperatures and very high pressures are limited not only as to the size of sheet formed but also as to the mesh size since the molten metal would cool before completely filling the mold.

In the sintering process the dry lubricant powder may decompose or vaporize at the sintering temperature, as would be the case with boric acid which melts at  $365^{\circ}$  F. with some decomposition and boils at  $572^{\circ}$  F. giving off water of crystallization and further decomposing. On the other hand, graphite powder has a melting point of substantially  $6380^{\circ}$  F. and would not be affected by the sintering heat so that the fine graphite particles would be maintained in the sintered mass of metal particles. Such would be the case with exfoliated vermiculite as well.

While we have illustrated and described only preferred embodiments of the present invention, it can be appreciated by those skilled in the art that various combinations of materials may be used, that various modifications of the process may be used, and that the apparatus used to perform the process may take various embodiments. All such as come within the scope of

the following claims are considered to be a part of our invention.

We claim:

1. The method of making metallic screen material comprising providing a block of material unaffected by temperatures capable of sintering the metal from which the screen material is made with depressions conforming to the mesh of the screen material, intimately associating comminuted metallic particles with a dry lubricating powder chosen from the class of materials represented by graphite, exfoliated vermiculite and boric acid in the proportion of substantially 98½% metal to 1½% dry lubricant, heaping a mass of the mixture on the shaped surface of the block, striking off the excess mixture, compressing the mixture into the depressions, and sintering the mixture in a non-oxidizing atmosphere.

2. The method of making metallic screen material comprising comminuting a metal of a high melting point and a metal of a low melting point, associating the comminuted metals intimately into a mixture consisting of a major proportion of the metal of high melting point, adding to the mixture a small proportion of powdered dry lubricant such as graphite exfoliated vermiculite, or boric acid, heaping a mass of the final mixture of metals and dry lubricant on the grooved surface of a mold, striking off the excess mixture above the grooves, compressing the material remaining in the grooves, repeating the operations of heaping the mixture on the grooved surface, striking off the excess, and compressing the material remaining in the grooves until the compressed mixture in the grooves is of the desired thickness, and sintering the material in the grooves of the mold in an oven having a non-oxidizing atmosphere therein maintained at a temperature between the melting points of the two metals.

3. The method of making fine-mesh metallic screen material comprising grooving a plane surface of a substantially infusible block in the shape of the screen material desired, comminuting an alloy of a metal of high melting point and structural strength having a relatively small proportion of metal of low melting point alloyed

therewith to an extent such that the particles of comminuted alloy are materially smaller in diameter than the dimensions of the grooves in the block, intimately associating with the comminuted alloy particles of dry powdered material such as graphite or the like, spreading the material over the surface of the block so as to fill the grooves of the block with such comminuted material, removing the excess material from the surface of the block, compressing the comminuted material in the grooves of the block, and sintering the material in a non-oxidizing atmosphere at a temperature below the melting point of the alloy but above the melting point of the metal of low melting point in the alloy.

4. Apparatus for forming screen material by sintering comminuted metal in a mold shaped to form such screen material comprising a mold of a substance infusible at a temperature capable of sintering the material of which the screen is made and having grooves in a surface thereof shaped to conform to the desired shape of screen material, and a press for compressing the comminuted metal into the grooves of the mold comprising a rubberous platen and means to effect relative movement between the grooved surface of the mold and said rubberous platen so as to compress the comminuted material into the grooves of the mold.

5. The method of making metallic screen material comprising providing a block of material unaffected by temperatures capable of sintering the metal from which the screen material is made with depressions conforming to the mesh of the screen material, intimately associating comminuted metallic particles with a dry lubricating powder chosen from the class of materials represented by graphite, exfoliated vermiculite and boric acid in the proportion of substantially 98½% metal to 1½% dry lubricant, heaping a mass of the mixture on the shaped surface of the block, removing the excess material from the surface of the block, compressing the mixture into the depressions, and sintering the mixture in a non-oxidizing atmosphere.

WILLIAM G. CALKINS.  
ROY E. BLUE.  
WARD W. MARVIN.